

L. Guild

Wringer Roll,

N<sup>o</sup> 36,494.

Patented Sep. 16, 1862.



Fig. 2.



Witnesses:  
D. C. Chapman  
Edward Mayhew  
Inventor:  
Lewis Guild  
by his attorney  
Samuel Cooper  
or Roach,

# UNITED STATES PATENT OFFICE.

LEWIS GUILD, OF DEDHAM, MASSACHUSETTS, ASSIGNOR TO WILLARD EVERETT & CO., OF SAME PLACE.

## IMPROVED ROLLERS FOR WASHING-MACHINES.

Specification forming part of Letters Patent No. 36,492, dated September 16, 1862.

*To all whom it may concern:*

Be it known that I, LEWIS GUILD, of Dedham, in the county of Norfolk and State of Massachusetts, have invented certain Improvements in Rolls for Clothes Wringing and Washing Machines, of which the following is a full, clear, and exact description, reference being had to the accompanying drawings, making part of this specification, in which—

Figure 1 is a perspective view of a roll for a clothes wringing machine without its covering of india rubber. Fig. 2 is a longitudinal section through the same.

In rolls for clothes wringing and washing machines, where an iron shaft passes lengthwise through the roll to give it strength and to form journals on which the roll turns, the iron is liable to be rusted by the water coming into contact with it and to stain the clothes; also, where a wooden roll is placed upon the iron shaft to be afterward covered with india-rubber, it is requisite that the wooden roll should be secured so that it cannot turn on the iron shaft.

The object of my present invention is to protect the iron shaft from corrosion, and at the same time to secure the wooden roll to the shaft; and my invention consists in casting onto the iron shaft a coating of metal, which will not stain the clothes when wet, and in connection therewith forming collars or heads, which serve to secure the wooden roll to the shaft and to protect the ends of the india-rubber covering, which is afterward applied to the roll.

I am aware that iron shafts have been washed or coated with tin, zinc, and alloys of metals to protect them from rust; but this washing or galvanizing of the shaft would not accomplish the end I have in view, which is not only to protect the shaft, but also to secure the wooden roll to the shaft and provide the collars which are necessary to protect the rubber covering of the roll.

That others skilled in the art may understand and use my invention, I will describe the manner in which I have carried it out.

In the said drawings, A is the iron shaft; B, the wooden roll through which the shaft is passed. The wooden roll is put on the shaft and these placed in a copper mold of the required form, and a coating, a, of zinc or other suitable metal or alloy is cast onto the iron shaft. At this same time there is cast a collar, C, at each end of the wooden roll, the metal entering and filling notches c made in the end of the wooden roll. This prevents the wooden roll from turning round on the shaft. To make the zinc or alloy adhere properly to the iron shaft, the shaft is first cleaned with weak sulphuric acid, and is then washed with a solution of zinc dissolved in muriatic acid. The copper mold is heated to prevent the chilling of the casting.

In some cases I intend to cast on only one of the collars C, and after the rubber covering has been applied to the outside of the wooden roll to solder on the other collar.

The wooden roll, after being secured to the shaft A, as described, is to be covered with india-rubber or other cloth wound around it and secured thereto, and on this basis is cemented the outer covering or tube of india-rubber. If the coating a is not sufficiently smooth it may be turned down in a lathe.

What I claim as my invention, and desire to secure by Letters Patent, as an improvement in clothes wringing and washing machines, is—

The coating a and collars C, cast onto the shaft A, whereby the journals are protected from rust, and the wooden roll B is secured to the shaft, substantially in the manner described.

LEWIS GUILD.

Witnesses:

ANSON MORSE,

NATHAN A. JOHNSON.